

# UNITED STATES PATENT OFFICE.

CARL BACHE-WIIG AND JOHN BACHE-WIIG, OF PORTLAND, MAINE; SAID JOHN BACHE-WIIG ASSIGNOR OF EIGHTY PER CENT OF HIS INTEREST TO SAID CARL BACHE-WIIG.

## PROCESS OF PREPARING FIBROUS PULP MATERIAL.

1,418,353.

Specification of Letters Patent. Patented June 6, 1922.

No Drawing.

Application filed August 21, 1920. Serial No. 405,087.

*To all whom it may concern:*

Be it known that we, CARL BACHE-WIIG and JOHN BACHE-WIIG, both citizens of the United States, residing at Portland, in the 5 county of Cumberland and State of Maine, have invented certain new and useful Improvements in Processes of Preparing Fibrous Pulp Material; and we do hereby declare the following to be a full, clear, and 10 exact description of the invention, such as will enable others skilled in the art to which it appertains to make and use the same.

This invention relates to a process of preparing fibrous paper pulp material suitable 15 for making print papers, from rye, wheat and other straws, and from similar fibrous cellulosic substances, and has for its object to improve certain of the somewhat similar processes which have been heretofore proposed.

With this and other objects in view the invention consists in the novel steps and combinations of steps constituting the process, all as will be more fully hereinafter 20 disclosed and particularly pointed out in the claims.

In order that the precise invention may be the more clearly understood it is said:— It is well known that papers of various 30 kinds have long since been made from materials such as those employed by us, but it is equally well known that up to the present time, print papers derived wholly from such materials have not been commercially supplied to the trade.

The reasons for this are partly as follows:—In the first place the yield of paper making fibres from such materials has been only about say 40% to 45% of the whole, 40 under the prior processes, and therefore, the cost of the resulting paper, for this reason alone, has been greatly increased. In the second place, the treatment of the straws has been such that the resulting fibres have 45 been too short to make a satisfactory print paper, although such short fibres have been satisfactorily used as filling materials when mixed with other and more expensive fibres.

In the third place, the chemicals employed 50 have been used in greater quantities and in stronger solutions than those found in our process, and they therefore have been so costly as to still further increase the total

cost of the final product. The result has been that prior to our invention, no one has 55 been able to commercially supply print papers and especially news print papers made wholly from straw like materials as are we.

In fact, in the case of news print paper the commercial requirements are so stringent that no one prior to us has even succeeded commercially in adding even say 10% or 20% of straw fibres to such paper.

In carrying out our invention, on the other hand, we avoid these various commercial objections and produce not only book print papers, but also news print papers, commercially, and wholly out of straw like materials, as will appear more fully hereinafter.

We accomplish these desirable results, 70 first, by giving to the straw like materials a relatively mild first or preliminary treatment. This has the effect of producing from the straw like material a quantity of pulp making fibre of from say 50% to 58%, or 75 higher, of the whole, thus largely increasing the amount of pulp material from the straw.

Second, owing to this relatively mild first treatment, and the later use of kollergangs and the introduction of other features to be 80 disclosed below, our fibres are found to be actually longer and very much stronger than are those which have been heretofore produced from straw like materials.

It therefore follows that the resulting paper produced by our process is of a much higher quality than that produced by prior processes.

Third, so weak are our solutions that we only use say about 25% to 30% of the weight 90 of the chemicals that have been heretofore employed in the making of paper from straw, and therefore, we save greatly in their cost, which very materially adds to the cheapness of the paper product.

Fourth, owing to the above mentioned relatively weak solutions, and mild first treatment, as well as to other features to be disclosed below, it is found that the cost of the plant, machinery, etc., is less than that 100 for the prior processes.

Fifth, and lastly, we eliminate the usual soda recovery plant, its attendant labor and cost to run, and owing to our said first treatment, and the kollergang treatment, the bulk 105 of the material treated is so reduced that it

is found our digestors may be say one half the capacity of the digestors heretofore employed and which treated the straw before it had been reduced in volume as it has been 5 in our case.

This latter still further reduces the cost of the finished product.

In carrying out this process, the straw is first cut into suitable lengths of say one inch 10 or more, and in any desired manner. It is then thoroughly screened to remove sand or other foreign substances. For the finer grades of paper, an air blast may be employed to clean the material more perfectly. 15 The cut material is now subjected to the above mentioned first or pre-treatment by packing the same into a closed container into which a bleach and softening, or disintegrating agent is introduced.

20 This said bleaching and softening agent is so chosen that the fibres are not injured or are not shortened as has been the case heretofore, and we find that we may use sulphur dioxide  $\text{SO}_2$  either in the form of a gas injected into the container or we may use a solution of common salt  $\text{NaCl}$ . If the gas is used it should not be at a pressure higher than say 2 to 10 pounds, but ordinarily we prefer not to exceed say 2 pounds pressure.

30 Instead of the gas, we of course may use  $\text{SO}_2$  in the form of a weak solution in which case, we prefer that it have a strength of not more than say one half of one per cent  $\text{SO}_2$ . In practice we have found, that the gas gives 35 the better results as it seems to penetrate the mass of material better.

In the case of making book paper pulp, or finer grades of paper pulp, we find that it is often desirable to use as much as 5 pounds 40 pressure of the gas. In other cases for special grades of paper, we may, of course, use higher pressures as will readily occur to those skilled in the art.

In the case of news print paper pulp, and 45 should a  $\text{SO}_2$  solution be employed, a strength of one half of one per cent  $\text{SO}_2$  is desirable, as above mentioned, but in the case of book paper pulps this strength may be correspondingly increased, or to say 1% or a 50 little higher.

Should a sodium chloride solution be used in this first or preliminary treatment, we find that the yield of fibres will be somewhat higher even than with the  $\text{SO}_2$  gas or solution, and we further find that the strength of the fibre is somewhat better because the salt seems to prevent, in some way, the sugar like constituents leaving the straw or cellulose before higher temperatures are reached, with 55 the result that the reaction taking place at said higher temperature is not so harsh or so weakening on the fibre as it would be if no salt were used.

In the making of news print pulp we pre- 65 fer to employ a solution of from 1% to 2%

of salt in this first or preliminary treatment, and in the case of making book print paper pulp we prefer to employ a solution of from say 3% to 4% of salt.

It is found in practice that straws differ 70 considerably in their composition and that some straws have considerably more silica than others. For those straws which are relatively high in silica, of course, a harsher chemical reaction is needed, to soften their 75 ligneous matter, than are straws which have a less silica content. Therefore, the time of treatment will depend somewhat upon the kind of straw used, and it will readily occur to those skilled in the art as to just how long 80 this preliminary treatment should last, but under ordinary conditions, it would last from say 12 to 18 hours.

During this preliminary treatment, however, and before any steam is applied, if  $\text{SO}_2$  85 gas has been employed the material should stand, subject to the action of said gas, for say 1 to 2 hours, whereupon a sufficient quantity of water is added to produce a solution substantially equal in strength of  $\text{SO}_2$  to that 90 above indicated, or a solution which will contain say about one half of 1 per cent of  $\text{SO}_2$ .

After this standing, steam at a pressure sufficient, if news print paper is to be made, 95 to produce a temperature of from say 50° to 60° C. or the temperature of the material may be otherwise suitably raised. This temperature is maintained in the case of news print paper for a period of from say 12 to 100 18 hours; in the case of book print, the steam will have a pressure sufficient to produce a temperature of from 80° to 90° C., and it will be maintained for a period of from 18 to 24 hours. In other words, ordinarily the 105 shorter the heating period the stronger and harder will be the resulting fibre. The longer the heating is continued the softer will be the fibre.

The length of the heating period will also, of course, depend somewhat upon 110 the character of the straw employed. Should  $\text{SO}_2$  gas not be used, but a solution of  $\text{SO}_2$  or a solution of  $\text{NaCl}$  be used in this said first, or pre-treatment, of the material, then the above mentioned heating is preferably 115 begun immediately upon the introduction of the material into the tank, and without allowing it to stand as is the case when the gas is employed.

The result of the foregoing preliminary 120 treatment is, as will be apparent from what has been above stated, that the ligneous matter present in the raw material is softened and to some extent dissolved, whereby the fibres of said material are not injured to any 125 substantial extent, and whereby they may be readily liberated by the succeeding steps of the process to be disclosed below.

In addition to this, the above mentioned softening agents naturally bleach the mate- 130

rial to a greater or less extent. Further, in the cases where the salt solutions are employed the amount of the yield of fibre is greatly increased owing to the fact that the 5 levulosic or other sugar like materials are left in the fibre and are not lost to the process as in the preceding cases, all as has been mentioned above. The fibres thus produced are found in practice to be abundantly strong 10 enough for making news print paper, and book paper. The above mentioned pre-treatment applies to all ordinary straws, and similar material, but when treating flax straw it is preferred to handle it in all cases 15 as if one is to make book paper pulp in the manner above disclosed. But, after this said first treatment is completed, it is preferred to wash it, and run it over kollergangs to loosen up its woody matter before it is 20 cooked.

The other straw may be treated in this manner also, and if it is so treated it will be found to require less time in cooking and also less chemicals. On the other hand, such 25 washing and kollergang treatment is not found to be essential in the handling of ordinary straws.

After the above mentioned preliminary treatment has been completed, the steam is 30 cut off and the liquor is withdrawn from the container. This liquor may be used over several times in treating fresh batches of straw material and when so used, it becomes quite rich in potash and ammonia, and these 35 reagents may be recovered if desired in any suitable manner.

The straw material remaining in the tank after the liquor has been drawn off is next 40 thoroughly washed with water and drained after which it is transferred to suitable digestors where it is further cooked in the presence of a bi-sulphite pulp forming solution. As above mentioned, the total volume 45 of the original straw has now been so reduced that the capacity of these digestors need not be more than about 50% of what they would be if this preliminary treatment had not been given the straw. This said solution may contain from say  $\frac{1}{10}\%$  to 1.1% 50 of caustic soda  $\text{NaOH}$ , or from say  $\frac{1}{10}\%$  to 1.1% of sodium carbonate  $\text{Na}_2\text{CO}_3$ , either or both mixed with  $\frac{1}{2}\%$  of sodium sulphate  $\text{Na}_2\text{SO}_4$ . We add this bisulphite forming 55 solution to the digestors immediately after putting in the straw, and then raise the temperature to  $125^\circ \text{C}$ . in about two hours time. After this temperature has been reached we next add a small amount of sodium chloride  $\text{NaCl}$  which amount usually will not exceed 60 5%. The function of this said sodium chloride at the temperature mentioned is that of a bleaching agent.

After the above mentioned bi-sulphite pulp forming solution has been thus added 65 to the digestors, as above stated, the temper-

ature of the mass is raised in any suitable manner to say from  $130^\circ \text{C}$ . to  $140^\circ \text{C}$ . and this said temperature is maintained for from say 4 to 8 hours, depending, again, upon the strength and hardness desired in the final 70 product, or as mentioned above, depending upon the difference in quality of the straw employed, or depending upon whether or not we are to make news print paper or book print paper. 75

All of these variations will readily occur to those skilled in the art. Of course, the sooner this said solution is added to the digestors the softer will be the final fibrous product, and vice versa. A somewhat higher 80 temperature than that above mentioned, or one up to say  $150^\circ \text{C}$ . may be employed if desired, but the higher the temperature used, the less stronger will be the resulting fibre and we have found that the ranges above 85 given are really the best to be employed in practice because they yield the greatest strength and greatest amount of fibre.

The cooking having been continued for about 4 hours in the case of news print 90 paper, and about 6 hours in the case of book print paper, the pulp mass is blown into a wash pit having a perforated double bottom through which the cooked liquor is withdrawn, whereupon said mass is washed and 95 then it is transferred to a kollergang apparatus to be ground.

As above intimated, it is an important feature of this invention that a kollergang is employed instead of any other type of 100 beating engine for it is found to act less harshly upon the fibre, and therefore, by its use it is possible to cook the pulp up to that predetermined point at which its maximum strength of fibre is still retained, and yet, 105 to so soften it as to permit a substantially complete disintegration thereof by the kneading action of the kollergang without injuring the fibre.

Stated in other language, the relatively 110 mild treatment to which the pulp has been subjected up to this point has resulted in producing an abnormally large percentage of the pulp from the straw and it has preserved a length of fibres and a strength of 115 fibres which has not been attained in any prior processes, in so far as we are aware.

It therefore remains to thoroughly disintegrate the fibre without destroying the same, and other workers in this art, in so far as we are able to learn, have not appreciated the importance of using a kollergang type of beating engine in connection with 120 said mild treatment in order to preserve the said strength and length of fibre just mentioned.

On the other hand, by combining these features we are enabled to produce print paper and book paper at a figure which heretofore has not been possible, and therefore, 1.)

we are enabled to put such papers on the market in competition with papers produced from other sources. After leaving the kollergang the pulp is screened and bleached 5 with chlorine or other suitable bleaching agent, in the usual manner, whereupon it is ready for the paper machine.

We have found by actual test that paper produced from straw pulp prepared in the 10 manner above stated is strong enough to sufficiently withstand being run through fast printing presses while at the same time, as stated above, it is commercially inexpensive enough to compete efficiently with the 15 usual news print and book print made from ground wood and chemical pulp. We have also found, in carrying out this process, that the cooking liquor which is withdrawn from the digestors at the end of the second step of 20 the process may be used with good results in place of the  $\text{SO}_2$  and the  $\text{NaCl}$  solutions employed in the first or preliminary step, but we prefer in most cases to employ two separate sets of solutions as has been described 25 above.

It is obvious that those skilled in the art may vary the details of the steps constituting the process without departing from the spirit of the invention, and therefore, we 30 do not wish to be limited to the above disclosure except as may be required by the claims.

What we claim is:—

1. The process of preparing paper pulp 35 material from straw like substances containing ligneous matter which consists in softening said substances with a chemical softening agent; subjecting said softened substance to a kollergang treatment; subjecting 40 the resulting mass to a digesting action in the presence of a pulp forming liquor containing mixed acid and alkali compounds; and then subjecting the mass to a second kollergang treatment, substantially as de- 45 scribed.

2. The process of preparing pulp paper material from straw like substances containing ligneous matter which consists in subjecting said substances to the action of a 50 bleaching and softening agent adapted to soften but not destroy the ligneous matter; subjecting the softened mass to a kollergang treatment; and digesting the resulting mass in the presence of a bisulphite pulp forming liquor, substantially as described.

3. The process of preparing paper pulp material from straw like substances containing ligneous matter which consists in heating said substances in the presence of a 55 bleaching agent adapted to soften but not destroy said ligneous matter; subsequently digesting the resulting mass in the presence of a bi-sulphite pulp forming liquor; and injecting into said mass a solution of sodium

chloride at a predetermined period of said 65 digestion, substantially as described.

4. The process of preparing paper pulp material from straw like substances containing ligneous matter which consists in heating said substances at a predetermined tem- 70 perature and for a predetermined time in the presence of a bleaching agent adapted to soften but not destroy said ligneous matter; subsequently digesting the resulting mass at a predetermined temperature for a predeter- 75 mined time in the presence of a bisulphite pulp forming liquor; injecting into said mass at a predetermined period of said di- gestion a solution of sodium chloride; and mechanically grinding said mass in a koller- 80 gang type of apparatus to form a pulp, sub- stantially as described.

5. The process of preparing paper pulp material from straw like substances containing ligneous matter which consists in heat- 85 ing said substances in the presence of a bleaching and softening agent of a strength too weak to injure the fibre, and to a tem- perature not exceeding  $100^{\circ}$  C. for a pre- determined period of time not exceeding 24 90 hours; withdrawing said softening agent and washing the mass; subsequently digest- ing said mass in the presence of a pulp form- ing liquor at a temperature not exceeding 160 $^{\circ}$  C. for a period of time not exceeding 95 10 hours; injecting into said mass a solution of sodium chloride at from 2 to 5 hours after the beginning of said digesting operation; withdrawing said pulp forming liquor and washing said mass; and mechanically grind- 100 ing said mass in a kollergang apparatus to form a pulp, substantially as described.

6. The process of preparing paper pulp material from straw containing ligneous matter which consists in heating said straw 105 in the presence of a solution of sodium chlo- ride to bleach and soften said ligneous mat- ter; subjecting the softened mass to a koller- gang treatment and subsequently digesting the resulting mass in the presence of a pulp 110 forming liquor containing sodium ions, sub- stantially as described.

7. The process of preparing paper pulp material from straw containing ligneous matter which consists in heating said straw 115 in the presence of a solution of sodium chlo- ride to bleach and soften said ligneous mat- ter; subsequently digesting the resulting mass in the presence of a pulp forming li- quor; and injecting a solution of sodium chlo- 120 ride into said mass at a predetermined point of said subsequent digestion, substantially as described.

In testimony whereof we affix our signatures.

CARL BACHE-WIIG.  
JOHN BACHE-WIIG.